

Patented July 3, 1923.

1,460,396

# UNITED STATES PATENT OFFICE.

JOSEPH N. WIGGIN, OF EAST ORANGE, NEW JERSEY, ASSIGNOR TO H. B. WIGGIN'S SONS COMPANY, OF BLOOMFIELD, NEW JERSEY, A CORPORATION OF NEW JERSEY.

PLASTER AND PROCESS OF CONTROLLING THE SETTING OF PLASTER, AN ACCELERATOR THEREFOR, AND PROCESS OF MAKING SUCH ACCELERATOR.

No Drawing.

Application filed April 29, 1920. Serial No. 377,707.

*To all whom it may concern:*

Be it known that I, JOSEPH N. WIGGIN, a citizen of the United States, residing at East Orange, in the county of Essex and State of New Jersey, have invented a certain new and useful Improvement in a Plaster and Processes of Controlling the Setting of Plaster, an Accelerator Therefor, and Processes of Making such Accelerator, of which the following is a specification.

The object of my invention has been to provide a plaster and a process of controlling the setting of plaster, an accelerator for plaster and a process of making such accelerator, whereby uniformity and definiteness of time of setting can be obtained; whereby the time of the setting of plaster, and particularly plaster of Paris, may be controlled; whereby crystallization throughout the mass shall be uniform; whereby greater cohesion and strength may be obtained than ordinarily; and whereby such results can be obtained economically, and to such ends my invention consists in a plaster and a process of controlling the setting of plaster, an accelerator therefor and a process of making such accelerator hereinafter specified.

My invention relates to plaster and particularly plaster of Paris, and I shall illustrate it by its application to plaster of Paris intended for dentists, but the illustrated embodiment is only to be regarded as typical of many possible embodiments, and my invention is not to be confined thereto.

For dental work, it is desirable that a powdered plaster be furnished, such that the time which it requires for the plaster to set can be controlled in advance, so that the setting will take place within, say, a given number of minutes. It is also desirable that such plaster shall have great cohesion and strength; that it may be made without the use of foreign substances; that the crystallization shall be uniform throughout the mass; and that it shall be economical.

My plaster has been proven by extensive experiments to possess these qualities.

Pure plaster of Paris is comparatively slow in setting when mixed with water. I provide an accelerator to hasten the setting. I desire to be able to sell a mixture, in powdered form, of the plaster of Paris with

the accelerator, which mixture shall remain in powdered form until it is desired to use it.

I have found that powdered plaster of Paris having a definite amount of water in a definite amount of plaster acts very favorably as an accelerator, and that where the amount of water in such accelerator is less than is necessary to solidify the entire mass, it will remain in powdered form when properly treated and can be mixed with the pure plaster of Paris without causing the latter to solidify.

I have found that by varying the proportion of water in the accelerator and by varying the proportion of accelerator in the mass of pure plaster of Paris, I can control the time of setting.

So far as known to me no one before me ever used as an accelerator plaster of Paris in which less water is present than is necessary to solidify the whole mass.

A further advantage of using an accelerator, in which the proportion of water is less than that necessary to solidify the whole mass, or to produce complete crystallization throughout the mass, is that a larger mass of accelerator is used than would be the case if the full amount of water necessary for such solidification were present, and this larger mass is more easily distributed uniformly throughout the mass of pure plaster of Paris than would be the case if the mass of accelerator were smaller. This more uniform distribution of the accelerator results in more uniform crystallization taking place when setting does occur. This more uniform crystallization gives greater cohesion and strength and it also gives that uniformity of time of setting which enables me to sell a mixture which will, with certainty, set in a definite desired time.

In preparing my accelerator, I preferably place a definite amount of powdered plaster of Paris in a mixing machine and sprinkle in a certain amount of water, stirring it all the time, say, for one hour. I then draw off the mixture of plaster and water and let it stand for a considerable time, say, one day, and finally pulverize it to a uniform size, for instance, a size that will pass through a 200-mesh sieve. As an

example of the proportion of water to plaster in my accelerator, one ounce of water may be used to one pound of plaster, by weight. In this proportion the accelerator is quite stable. By increasing the proportion of water the accelerator will work more rapidly.

- My process of forming the accelerator solves the problem of getting a definite amount of water in a definite amount of plaster and still keeping it in powdered form. While I have given the reasons and effects involved in my invention, as I suppose them to be, I do not vouch for them as being correct, nor as being the only reasons or effects which are involved. Extensive experimentation has shown that my accelerator and plaster very effectually accomplish the objects in view.
- My mixture of plaster and accelerator can not only be used without other substances, but desirable mixtures with other substances can be made. For instance, cement may be added in varying proportions, say, two parts of plaster to one part of cement. Or magnesium oxide or magnesium chloride or a mixture of both may be added to my mixture of plaster of Paris and accelerator. Many other mixtures are possible.

Throughout the claims by the terms "water" and "water of crystallization", etc., is meant water which causes the plaster to set as distinguished from water which necessarily enters into the molecule of plaster to constitute the latter before setting.

I claim:

1. A plaster of Paris composition comprising a mass of powdered plaster of Paris substantially without water and a second mass of plaster of Paris having water mixed therewith, but in less proportion than would be sufficient to solidify said second mass.
2. A plaster of Paris composition comprising powdered plaster of Paris substantially without water of crystallization, a powdered plaster of Paris having water therein of an amount less than sufficient to solidify said latter powdered plaster of Paris.
3. A process of controlling the setting of plaster consisting in mixing therewith a mass of plaster having fluid of crystallization but of less amount than sufficient to solidify said mass, and proportioning said mass of plaster to the body of plaster, whose setting is to be controlled, according to the time of setting desired.
4. A process of controlling the setting of plaster of Paris consisting in mixing therewith a mass of plaster of Paris having

water therein but of less amount than sufficient to solidify said mass.

5. A process of controlling the setting of plaster of Paris consisting in mixing therewith a definite amount of accelerator, which accelerator consists of plaster of Paris having water therein but of less amount than sufficient to solidify the mass of said accelerator.

6. A process of making an accelerator for a settable plaster consisting in mixing water with a mass of settable plaster to an amount less than sufficient to set said mass of plaster.

7. A process of making an accelerator for plaster of Paris consisting in mixing with a mass of plaster of Paris an amount of water less than sufficient to solidify said mass.

8. A process of making an accelerator for plaster of Paris consisting in mixing with a mass of powdered plaster of Paris a proportion of water less than the amount sufficient to solidify said mass and afterwards pulverizing said mass.

9. A process of making an accelerator for plaster of Paris consisting in mixing with a mass of powdered plaster of Paris a definite amount of water less than the amount sufficient to solidify said mass and afterwards pulverizing said mass.

10. A process of making an accelerator for plaster of Paris consisting in mixing water with a mass of powdered plaster of Paris, said water being in less proportion than sufficient to solidify said mass, permitting said mixture to stand until said water has been taken up and then pulverizing the mass.

11. A process of making an accelerator for plaster of Paris consisting in mixing water with a mass of powdered plaster of Paris, said water being in less proportion than sufficient to set the said mass and agitating said mass while mixing the water therewith.

12. A process of making an accelerator for plaster of Paris consisting in sprinkling into a mass of plaster of Paris an amount of water less than sufficient to set said mass of plaster.

13. A process of making an accelerator for plaster of Paris consisting in sprinkling into a mass of plaster of Paris an amount of water less than sufficient to set said mass of plaster and agitating said mass while sprinkling and mixing said water therewith.

In testimony that I claim the foregoing, I have hereunto set my hand this 27th day of April, 1920.

JOSEPH N. WIGGIN.